

Aug. 26, 1930.

E. C. GASKILL

1,773,779

METHOD OF REDUCING ZINC ORE AND THE PRODUCT OBTAINED THEREBY

Filed Dec. 17, 1926



INVENTOR,  
Earl C. Gaskill

BY

ATTORNEY,  
Abel L. Beaman

## UNITED STATES PATENT OFFICE

EARL C. GASKILL, OF RED BANK, NEW JERSEY, ASSIGNEE TO ST. JOSEPH LEAD COMPANY, OF NEW YORK, N. Y., A CORPORATION OF NEW YORK

METHOD OF REDUCING ZINC ORE AND THE PRODUCT OBTAINED THEREBY

Application filed December 17, 1926. Serial No. 155,471.

This invention relates generally to the electric reduction of zinc ore and more particularly to the direct production of metallic zinc by the smelting of loose ore in furnaces 5 of the electric resistor type.

It is well known and has been the standard practice for a long period of time to reduce zinc ore by a distillation process which comprises the heating of small batches of ore in 10 clay retorts in order to produce vaporization of the zinc content thereof and the subsequent condensing of the zinc vapors in relatively small condensing chambers attached to the mouths of the retorts.

15 This practice, although it has gone into universal and extensive use, is open to the objection that it is costly to carry out because of the great expense of labor involved in attending to the small batch type retorts and 20 also because of the expense involved in replacing the retorts which are easily broken.

It is a general object of the present invention to provide a process for the reduction of zinc ore and the direct production of metallic 25 zinc with little or no passing of the zinc through an intermediate vapor stage as it is converted from the oxide, or other form in which it exists in the ore, to the form of metal or spelter.

30 I have found in the course of experiments carried on for the purpose of invention that by heating a column of loose zinc ore intermixed with carbonaceous material by passing through the column an electric current, the 35 zinc content of the ore can be converted directly into metallic zinc which issues from the bottom of the furnace without having to pass through a specially built condensing chamber.

40 A suitable apparatus for carrying out this process is shown in the single diagrammatic view which constitutes a drawing illustrating the invention.

Referring to the drawing a furnace 10 of 45 the vertical shaft type is shown in which are mounted a pair of annular electrodes 11 and 12 in a vertically separated position such that current flowing between the electrodes passes through material filling the core or chamber of the furnace. This furnace structure

follows in a general way that shown in my prior application, Serial No. 148,801, filed November 17, 1926.

The furnace is constructed of suitable material to retain the heat developed therein and is preferably equipped at its upper end with a superheater 14 in which material about to enter the reducing zone 13 is brought up to a temperature such that reduction can immediately begin when current is applied to the heated material. The charge is heated in a preheater to a temperature of at least 600° C., and preferably from 750° to 800° C. The superheater 14 may be operated with a gas or oil burner such as shown at 15.

A heater 16 is also employed for heating the material to a temperature such as will drive out the moisture content, the temperature being somewhat lower than that to which the material is subjected in the superheater 14 in order not to injure metal parts.

A gate or valve 17 is operated by a motor not shown which is in turn controlled by electrodes 18 to automatically feed material through the passage 19 into the upper end of the superheater 14 when the level of material has fallen below the upper of the two electrodes 18. A hinged cover plate 20 is provided at the upper end of the furnace shaft through which access may be had to the 50 furnace chamber for any purpose.

The lower end of the furnace structure is provided with a cooling chamber 21 which may be formed of a simple metal cylinder in which the contents are cooled by the contact 55 of air with the external surface of the cylinder. If desired, a water cooling jacket may be applied to the member 21 as will be clear.

The lower end of the cooling chamber 21 delivers material to the upper surface of a 60 perforated plate 22 which closes the upper end of a shallow receptacle 23 in which molten metal contained in the material issuing from the cooling chamber 21 finds its way. The receptacle 23 is mounted on the 65 upper end of a rotatable shaft 24 and it will be seen that material deposited on the upper plate 22 is subjected to a separating operation by which the molten metallic content passes into the receptacle 23 and through an 700



ture at which the zinc ore is reduced to metal but below the temperature at which the metal is substantially vaporized, and separating the liquid metallic zinc and solid residue thereby produced.

5 2. A process for producing metallic zinc directly from ore which comprises heating a mixture of sintered zinc ore and carbonaceous material, by means of an electric current 10 passed therethrough, to a temperature at which the zinc ore is reduced to metal but below the temperature at which the metal is substantially vaporized, and separating the liquid metallic zinc and solid residue thereby 15 produced.

EARL C. GASKILL.

20

25

30

35

40

45

50

55

60

65